

## UNITED STATES PATENT OFFICE

2,248,091

PROCESS OF PRODUCING FAST DYEINGS  
AND THE DYED FIBER OBTAINED THEREBY

Werner Kirst, Konigsten in Taunus, and Wolfgang Alt and Hans Krzikalla, Ludwigshafen-on-the-Rhine, Germany, assignors to General Aniline &amp; Film Corporation, a corporation of Delaware

No Drawing. Application September 24, 1938, Serial No. 231,594. In Germany September 24, 1937

9 Claims. (Cl. 8—21)

The present invention relates to the production of fast dyeings and to the dyed fiber obtained thereby.

We have found that dyeings of good properties of fastness, especially of high fastness to wet processing may be obtained by applying to the textile fiber in a feebly alkaline, neutral or feebly acid bath a water-soluble azo-dyestuff containing in the molecule an amino-group capable of being diazotized and a hydroxyl group rendering coupling possible, then diazotizing the dyestuff on the fiber and causing it to combine with itself. The self-coupling may be performed or completed, for instance, by adding to the diazo-bath an agent neutralizing the acid or having an alkaline action, after the diazotization is finished, or by passing the goods through a bath having an alkaline action.

The fastness properties of the dyeings obtained are surprisingly good, especially when considering that by the coupling the number of the solubilizing groups remains practically the same with respect to the molecular weight, whereas the improvement of the fastness properties of the known diazotizing- and developing-dyestuffs is produced by increasing the molecule, the number of the solubilizing groups remaining the same. As far as the dyestuffs produced on the fiber contain groups capable of forming metal complex compounds, such as hydroxyl, carboxyl or alkoxy groups in ortho-position to the azo-group, the fastness properties of the dyeings may be improved by an after-treatment with agents yielding metal. There may also be used as parent materials water-soluble azo-dyestuffs containing already metal in complex union.

By the new process it is possible to obtain, in a relatively simple way and without the fiber being damaged, fast dyeings on animal fibers or on natural or artificial cellulose fibers and, especially, on mixed fibers. It is surprising that the dyeings obtained by diazotizing the azo-dyestuffs on the fiber and coupling them in a feebly alkaline bath have a very good fastness to rubbing, without the intermediate rinsing baths, usually applied in dyeing with diazotizing dyestuffs between dyeing and diazotizing or between diazotizing and coupling being inserted whereby the dyeing process is greatly facilitated for the dyer.

Mixed fibers from artificial silk staple fiber and wool have, for instance, hitherto been dyed by applying to the mixed fiber, in a neutral bath, a diazotizing dyestuff and an acid wool dyestuff stable to diazotizing, then rinsing the material,

10 diazotizing, rinsing and developing the dyeing by means of a developer, such as beta-naphthol. This process may now be conducted in a considerably simpler way by using according to the present invention an azo-dyestuff having an affinity for cotton and containing an amino-group capable of being diazotized and a hydroxyl group rendering coupling possible, applying this dyestuff, together with an acid wool dyestuff stable to diazotizing, to the mixed fiber, diazotizing the dyestuff on the fiber, centrifuging the material and causing self-coupling by addition of some alkali to the subsequent rinsing bath, and then rinsing again.

15 Mixtures of animal fibers, such as wool, with artificial or natural cellulose fibers may also be dyed uniformly with one dyestuff by using water-soluble azo-dyestuffs containing an amino-group capable of being diazotized and a hydroxyl group rendering coupling possible, which have an affinity for both kinds of fibers. Practically tone-in-tone dyeings may, for instance, be obtained on mixtures of wool and viscose staple fiber or other regenerated celluloses by applying to the fiber, 20 in a feebly alkaline, neutral or feebly acid bath at raised temperature, for instance, a water-soluble azo-dyestuff of the following general constitution:



25 wherein R<sub>1</sub> stands for an aryl radical or a grouping of several aryl radicals which may be connected with each other by members, such as —N=N—, —NH—CO—, —NH—CO—NH—, —CH<sub>2</sub>—, —NH— and the like, and R<sub>2</sub> means hydrogen or a substituent, then squeezing or centrifuging the material, diazotizing the dyestuff on the fiber and developing the dyeing by treatment with an agent having a feebly alkaline action. In an analogous manner the water-soluble azo-dyestuffs obtainable by coupling a diazotized 30 amino-naphthol or amino-naphthol-sulphonic acid with an aminophenyl-methyl-pyrazolone or a substitution product thereof may, for instance, also be developed on the fiber with production of fast dyeings.

35 Furthermore, mixed fibers from wool and vis-

cose staple fiber or cuprammonium staple fiber may be dyed by the new process by applying to the fiber a water-soluble mono-azo-dyestuff containing an amino-group capable of being diazotized and a hydroxyl group rendering coupling possible together with a water-soluble dis- or poly-azo-dyestuff having an affinity for cotton and containing an amino-group capable of being diazotized and a hydroxyl group rendering coupling possible, then diazotizing both dyestuffs on the fiber and causing self-coupling by a treatment with an agent having an alkaline action. If the dyestuffs are suitably selected, tone-in-tone dyeings or mixed shades may thus be obtained.

The preceding statements characterize some possibilities of applying the new process. The temperature during the dyeing process depends on the class of dyestuffs used and on the desired effect. The diazotization on the fiber is preferably conducted in the cold or at a slightly raised temperature, by means of a nitrite and an acid, such as hydrochloric acid, sulfuric acid, formic acid and the like, wetting agents being, if desired, added to the bath, in order to improve the wetting efficiency in the subsequent bath having an alkaline action. The dyeing is developed either in a fresh bath by means of dilute feeble alkalies, such as ammonia, or by means of inorganic salts having an alkaline action, such as sodium carbonate, sodium bicarbonate, potassium carbonate or organic bases having an alkaline action or the salts thereof having an alkaline action. The diazotizing bath may also be neutralized by addition of an alkali and the dyeing may be developed by rendering this bath feebly alkaline. The fastness properties of the dyeings may be improved by a subsequent treatment with washing agents, such as soap or the reaction product from 10 mols of ethylene-oxide and 1 mol of isoocetyl-phenol.

The following examples illustrate the invention, the parts being by weight, unless otherwise stated:

(1) 1 kg. of mixed yarn from 30 parts of viscose staple fiber and 70 parts of wool is treated, for one hour at 75° C., with 50 grams of the sodium salt of the azo-dyestuff, obtainable by coupling diazotized 1-amino-2-chloro-4-nitrobenzene in an acid medium with 2-amino-5-hydroxynaphthalene-7-sulfonic acid and subsequently reducing the product obtained, and 80 grams of ammonium sulfate in 24 liters of water. 600 grams of sodium sulfate dissolved in 6 liters of cold water are then added and the material is treated for a further hour at 60° C., centrifuged and introduced into a cold bath containing per 30 liters of water

|                                      |       |     |
|--------------------------------------|-------|-----|
| Sodium nitrite                       | grams | 35  |
| Sodium dibutyl-naphthalene-sulfonate | grams | 30  |
| Sodium sulfate                       | do    | 500 |
| Hydrochloric acid of 20° Bé          | cc    | 90  |

After diazotization for half an hour the material is centrifuged and developed for half an hour in a bath containing per 30 liters of cold water

|                                                            |       |    |
|------------------------------------------------------------|-------|----|
| Ammonia of 25 per cent. strength                           | cc    | 80 |
| Reaction product from ethylene-oxide and octodecyl alcohol | grams | 10 |

The material is rinsed cold, treated at 40° C. with a solution containing per liter 0.1 gram of the reaction product from 10 mols of ethylene-oxide and 1 mol of isoocetyl-phenol and 0.5 gram of

sodium carbonate, rinsed cold and hot and then dried. A black dyeing of good fastness properties is obtained.

(2) 1 kg. of mixed yarn from 30 parts of cuprammonium staple fiber and 70 parts of wool is treated for one hour at 85° C. with 24 liters of water containing 30 grams of the sodium salt of the azo-dyestuff obtainable by coupling diazotized 2-amino-5-hydroxynaphthalene-7-sulfonic acid with 1-(4'-aminophenyl)-3-methyl-5-pyrazolone. 600 grams of sodium sulfate dissolved in 6 liters of cold water are then added and the material is treated for another hour at about 70° C., centrifuged, diazotized and developed as indicated in Example 1, rinsed cold and hot and then dried. A dark-brown dyeing of good fastness properties is obtained.

(3) 1 kg. of a mixed fabric from 50 parts of viscose staple fiber and 50 parts of wool is treated, for one hour at 85° C. to 90° C., with 24 liters of water containing 80 grams of ammonium sulfate and 30 grams of the sodium salt of the azo-dyestuff obtainable by coupling diazotized 1-amino-4-(4'-nitrobenzoyl)-aminobenzene, in an acid medium with 2-amino-5-hydroxynaphthalene-7-sulfonic acid and subsequently reducing the product obtained, and 30 grams of the sodium salt of the azo-dyestuff obtainable by coupling diazotized 2-amino-8-hydroxynaphthalene-6-sulfonic acid with 1-amino-2-methoxy-5-methylbenzene, diazotizing again and coupling the diazo compound in an alkaline medium with 2-amino-8-hydroxynaphthalene-6-sulfonic acid. 600 grams of sodium sulfate dissolved in 6 liters of cold water are then added and the material is treated for another hour at 70° C. to 75° C., then centrifuged, diazotized and developed in an ammoniacal bath as indicated in Example 1, rinsed and dried.

40 A black dyeing of good fastness properties is obtained.

(4) A mixed fabric consisting of 30 per cent of viscose artificial silk and 70 per cent. of wool is treated, for half an hour at 90° C., in a bath containing 5 per cent. of the disazo-dyestuff of the following formula:



(obtainable by combining one mol of tetrazotized 4,4'-diaminodiphenyl with one mol of 2-amino-5-hydroxynaphthalene-7-sulfonic acid in an alkaline solution and one mol of 1,5-dihydroxynaphthalene-3,7-disulfonic acid), 20 per cent. of Glauber's salt being added to the bath. 5 per cent. of acetic acid are then added and the material is dyed for another half hour at 90° C. (The percents are calculated upon the weight of the fiber.) After rinsing for a short time, the fabric is diazotized for half an hour in a cold bath containing per liter 2 grams of sodium nitrite, 5 cc. of hydrochloric acid of 35 per cent. strength and 20 grams of sodium chloride, rinsed again and then treated for a quarter of an hour at room temperature in a bath containing per liter 2 grams of sodium bicarbonate and subsequently soaped. The coupling may also be effected in the diazotizing-bath itself by adding thereto sodium bicarbonate until the reaction is feebly alkaline. By this treatment the direct red-violet tint turns to a deep brown-violet shade of considerably better fastness properties.

(5) A skein or fabric from viscose artificial silk is dyed for one hour at 80° C. with 5 per cent of the dyestuff of the following constitution:



(obtainable by combining mono-diazotized 2,6-

dichloro-1,4-diaminobenzene in an acid solution with 2-amino-5-hydroxynaphthalene-7-sulfonic acid, while adding 20 per cent. of sodium chloride. (The percents are calculated upon the weight of the fiber.) A reddish-brown dyeing is obtained which, by the process of diazotizing and coupling on the fiber as described in Example 4, turns to a violetish-brown tint of considerably improved fastness properties.

If the above-named dyestuff is exchanged for the following dyestuff:



yields, when diazotized and coupled, a violet-blue shade, the fastness properties of which are essentially improved with respect to the direct dyeing.

The dyestuff of the following constitution:



is less suitable for the production of uniform dyeings on mixed fabrics, since the shades of the after-treated dyeings on wool and viscose artificial silk do not completely correspond which, however, may be desirable under certain circumstances for the production of effects. This dyestuff may also be applied to cotton or viscose artificial silk and the dyeing obtained may then be converted by after-treatment into a red-violet shade of considerably enhanced fastness properties.

(7) A mixed fabric consisting of 30 per cent. of viscose artificial silk and 70 per cent. of wool is dyed for 1 hour at 70° C. with 50 per cent of sodium sulfate and 8 per cent. of the dyestuff of the following constitution:



(obtainable by coupling diazotized 1-amino-4-acetylaminobenzene in an alkaline solution with 2-amino-5-hydroxynaphthalene-7-sulfonic acid, transforming the product obtained into the 2-hydroxynaphthalene-3-carboxylic acid amide and splitting off the acetyl-group, or by coupling diazotized p-nitraniline with 2-amino-5-hydroxynaphthalene-7-sulfonic acid, transforming the product obtained into the 2-hydroxynaphthalene-3-carboxylic acid amide and subsequently



reducing the nitro-group). The material is then squeezed or rinsed for a short time and subsequently treated for half an hour in a diazotizing-bath containing per liter 2 grams of sodium nitrite, 5 cc. of hydrochloric acid of 35 per cent. strength and 20 grams of sodium chloride. The material is rinsed again for a short time and then treated for a quarter of an hour in a bath containing per liter 2 grams of sodium bicarbonate.

The coupling may also be effected in the diazotizing-bath itself by adding sodium bicarbonate until the reaction is feebly alkaline.

Fast black dyeings are obtained by using under the same conditions the dyestuff of the following constitution:



(obtainable by coupling diazotized 1-amino-4-acetylaminonaphthalene in an alkaline solution

with 1-amino-8-hydroxynaphthalene-3,6-disulfonic acid, transforming the product obtained into the 2-hydroxynaphthalene-3-carboxylic acid amide and subsequently splitting off the acetyl-group.

Fast black-brown tints are obtained by using in an analogous manner the dyestuff of the following constitution:

10



(obtainable by coupling diazotized 5-amino-4-methoxy-2-nitro-1-methylbenzene in an alkaline solution with 2-amino-5-hydroxynaphthalene-7-sulfonic acid, transforming the product obtained into the 2-hydroxynaphthalene-3-carboxylic acid amide and subsequently reducing the nitro-group). The fastness to light of the dyeings may be improved by a treatment with salts of metals capable of forming complex compounds (for instance copper salts) on the fiber before or after diazotizing and coupling or during the coupling reaction. It is also possible to start directly from the metal complex compounds of the dyestuff made in substance.

The following table illustrates the shades of a number of further dyeings obtainable by this invention:

|    | Parent dyestuff                                                                                                                                                                             | Shade on mixed fibers from artificial silk staple fiber and wool                 |
|----|---------------------------------------------------------------------------------------------------------------------------------------------------------------------------------------------|----------------------------------------------------------------------------------|
| 1  | 1-amino-4-nitrobenzene $\xrightarrow{\text{acid}}$ 2-amino-5-hydroxynaphthalene-7-sulfonic acid, reduced                                                                                    | Reddish-black.                                                                   |
| 2  | 1-amino-3-nitrobenzene $\xrightarrow{\text{acid}}$ 2-amino-5-hydroxynaphthalene-7-sulfonic acid, reduced                                                                                    | Garnet-red-brown.                                                                |
| 3  | 1-amino-2-hydroxy-4-nitrobenzene $\xrightarrow{\text{acid}}$ 2-amino-5-hydroxynaphthalene-7-sulfonic acid, reduced                                                                          | Black-violet, after-treated with a copper compound: black, after-chromed: black. |
| 4  | 1-amino-2-methoxy-4-nitrobenzene $\xrightarrow{\text{acid}}$ 2-amino-5-hydroxynaphthalene-7-sulfonic acid, reduced                                                                          | Black, after-treated with a copper compound: black, after-chromed: black.        |
| 5  | 1-amino-4-nitrobenzene $\xrightarrow{\text{alkaline}}$ 2-amino-5-hydroxynaphthalene-7-sulfonic acid $\xrightarrow{\text{acid}}$ 2-phenylamino-5-hydroxynaphthalene-7-sulfonic acid, reduced | Black-violet, after-treated with a copper compound: black-violet.                |
| 6  | 1-amino-2-chloro-4-nitrobenzene $\xrightarrow{\text{acid}}$ 2-amino-5-hydroxynaphthalene-7-sulfonic acid, benzoylated and reduced                                                           | Reddish-black.                                                                   |
| 7  | 1-amino-3-nitrobenzene $\xrightarrow{\text{acid}}$ 2-phenylamino-5-hydroxynaphthalene-7-sulfonic acid, reduced                                                                              | Reddish-brown.                                                                   |
| 8  | 1-amino-4-nitrobenzene $\xrightarrow{\text{acid}}$ 2-amino-5-hydroxynaphthalene-7-sulfonic acid, benzoylated and reduced                                                                    | Reddish-black.                                                                   |
| 9  | 1-amino-3-nitrobenzene $\xrightarrow{\text{acid}}$ 2-amino-5-hydroxynaphthalene-7-sulfonic acid, benzoylated and reduced                                                                    | Brown-red.                                                                       |
| 10 | 2-amino-5-hydroxynaphthalene-7-sulfonic acid $\xrightarrow{\text{acid}}$ 1-(3'-aminophenyl)-3-methyl-5-pyrazolone                                                                           | Covered red.                                                                     |
| 11 | 2-amino-5-hydroxynaphthalene-7-sulfonic acid $\xrightarrow{\text{acid}}$ 1-(3'-aminophenyl)-5-pyrazolone-3-carboxylic acid                                                                  | Bordeaux.                                                                        |
| 12 | 2-amino-5-hydroxynaphthalene-6-sulfonic acid $\xrightarrow{\text{acid}}$ 1-(3'-aminophenyl)-5-pyrazolone-3-carboxylic acid                                                                  | Red-brown.                                                                       |
| 13 | 1-amino-5-hydroxynaphthalene-7-sulfonic acid $\xrightarrow{\text{acid}}$ 1-(4'-aminophenyl)-3-methyl-5-pyrazolone                                                                           | Brownish garnet.                                                                 |
| 14 | 1-amino-5-hydroxynaphthalene-7-sulfonic acid $\xrightarrow{\text{acid}}$ 1-(3'-aminophenyl)-3-methyl-5-pyrazolone                                                                           | Covered red.                                                                     |
| 15 | 1-amino-5-hydroxynaphthalene-7-sulfonic acid $\xrightarrow{\text{acid}}$ 1-(3'-aminophenyl)-5-pyrazolone-3-carboxylic acid                                                                  | Bordeaux red.                                                                    |
| 16 | 1-amino-5-hydroxynaphthalene $\xrightarrow{\text{acid}}$ 1-(3'-aminophenyl)-5-pyrazolone-3-carboxylic acid                                                                                  | Do.                                                                              |
| 17 | 2-amino-8-hydroxynaphthalene-6-sulfonic acid $\xrightarrow{\text{acid}}$ 1-amino-3,5-dimethylbenzene, condensed with 3-nitro-4-methoxybenzoylchloride and reduced                           | Do.                                                                              |
| 18 | 2-amino-5-hydroxynaphthalene-7-sulfonic acid $\xrightarrow{\text{acid}}$ 1-amino-3,5-dimethylbenzene, condensed with 3-nitro-4-methoxybenzoylchloride and reduced                           | Vivid red-brown.                                                                 |
| 19 | 2-amino-5-hydroxynaphthalene $\xrightarrow{\text{acid}}$ 1-(3'-aminophenyl)-5-pyrazolone-3-carboxylic acid                                                                                  | Orange-brown.                                                                    |
| 20 | 2-amino-8-hydroxynaphthalene $\xrightarrow{\text{acid}}$ 1-(3'-aminophenyl)-5-pyrazolone-3-carboxylic acid                                                                                  | Copper-brown.                                                                    |
| 21 | 1-amino-5-hydroxynaphthalene-7-sulfonic acid $\xrightarrow{\text{acid}}$ 1-amino-3-methyl-6-methoxybenzene, condensed with 4-nitrobenzoylchloride and reduced                               | Bordeaux.                                                                        |
| 22 | 1-amino-5-hydroxynaphthalene-7-sulfonic acid $\xrightarrow{\text{acid}}$ 1-amino-3-methyl-6-methoxybenzene, condensed with 3-nitro-4-methoxybenzoylchloride and reduced                     | Brown.                                                                           |
| 23 | 2-(4'-aminobenzoyl-4'-aminobenzoyl-amino)-5-hydroxynaphthalene-7-sulfonic acid $\xrightarrow{\text{acid}}$ 1-amino-2-methoxy-5-methylbenzene                                                | Do.                                                                              |
| 24 | 2-amino-5-hydroxynaphthalene-7-sulfonic acid $\xrightarrow{\text{acid}}$ 1-amino-3-methyl-6-methoxybenzene, condensed with 4-nitrobenzoylchloride and reduced                               | Garnet.                                                                          |
| 25 | 2-amino-5-hydroxynaphthalene-7-sulfonic acid $\xrightarrow{\text{acid}}$ 1-amino-3-methyl-6-methoxybenzene, condensed with 3-nitro-4-methoxybenzoylchloride and reduced                     | Brown.                                                                           |
| 26 | 2-amino-8-hydroxynaphthalene-6-sulfonic acid $\xrightarrow{\text{acid}}$ 1-(3'-aminophenyl)-3-methyl-5-pyrazolone                                                                           | Brown-red.                                                                       |
| 27 | 2-amino-7-hydroxynaphthalene $\xrightarrow{\text{acid}}$ 1-(3'-aminophenyl)-5-pyrazolone-3-carboxylic acid                                                                                  | Red.                                                                             |
| 28 | 2-amino-8-hydroxynaphthalene-6-sulfonic acid $\xrightarrow{\text{acid}}$ 1-aminonaphthalene $\xrightarrow{\text{acid}}$ Cleve's acid                                                        | Dark-brown.                                                                      |
| 29 | 1-amino-7-hydroxynaphthalene $\xrightarrow{\text{acid}}$ Cleve's acid $\xrightarrow{\text{acid}}$ 2-amino-8-hydroxynaphthalene-6-sulfonic acid                                              | Dark-blue.                                                                       |
| 30 | 1-amino-4-nitrobenzene $\xrightarrow{\text{acid}}$ 1-amino-2-methoxy-5-methylbenzene $\xrightarrow{\text{acid}}$ 2-amino-5-hydroxynaphthalene-7-sulfonic acid, reduced                      | Dark-brown.                                                                      |

|    | Parent dyestuff                                                                                                                                                 | Shade on mixed fibers from<br>artificial silk staple fiber<br>and wool |
|----|-----------------------------------------------------------------------------------------------------------------------------------------------------------------|------------------------------------------------------------------------|
| 31 | 2-amino-8-hydroxynaphthalene-6-sulfonic acid → 1-(3'-aminophenyl)-3-methyl-5-pyrazolone → Cleve's acid.                                                         | Brown.                                                                 |
| 32 | 2-amino-5-hydroxynaphthalene-7-sulfonic acid → 1-amino-naphthalene → Cleve's acid.                                                                              | Do.                                                                    |
| 33 | 2-amino-5-hydroxynaphthalene-7-sulfonic acid → 1-amino-3,5-dimethylbenzene → Cleve's acid.                                                                      | Do.                                                                    |
| 34 | 2-amino-8-hydroxynaphthalene-6-sulfonic acid → 1-amino-3,5-dimethylbenzene → 2-(4'-aminobenzoyl-amino)-8-hydroxynaphthalene-6-sulfonic acid.                    | Dark-violet.                                                           |
| 35 | 2-amino-8-hydroxynaphthalene-6-sulfonic acid → 1-amino-3,5-dimethylbenzene → 2-(4'-aminobenzoyl-amino)-5-hydroxynaphthalene-7-sulfonic acid.                    | Do.                                                                    |
| 36 | 2-amino-8-hydroxynaphthalene-6-sulfonic acid → 1-amino-3,5-dimethylbenzene → Cleve's acid.                                                                      | Dark-brown.                                                            |
| 37 | 2-amino-5-hydroxynaphthalene-7-sulfonic acid → meta-amino-acetanilide.                                                                                          | Black-violet.                                                          |
| 38 | 2-(4"-aminobenzoyl-4'-aminobenzoyl-amino)-5-hydroxynaphthalene-7-sulfonic acid → Cleve's acid.                                                                  | Dark-brown.                                                            |
| 39 | 2-(4"-aminobenzoyl-4'-aminobenzoyl-amino)-5-hydroxynaphthalene-7-sulfonic acid → 1-amino-8-hydroxynaphthalene-3,6-disulfonic acid.                              | Violet-brown.                                                          |
| 40 | 2-amino-8-hydroxynaphthalene-6-sulfonic acid → 1-amino-2-methoxy-5-methylbenzene → 2-amino-5-hydroxynaphthalene-7-sulfonic acid.                                | alkaline<br>Reddish blue-black.                                        |
| 41 | 2-amino-8-hydroxynaphthalene-6-sulfonic acid → 1-amino-2-methoxy-5-methylbenzene → Cleve's acid.                                                                | alkaline<br>Dark-brown.                                                |
| 42 | 2-amino-8-hydroxynaphthalene-6-sulfonic acid → 1-amino-2-methoxy-5-methylbenzene → 1-amino-8-hydroxynaphthalene-5-sulfonic acid.                                | alkaline<br>Black-violet.                                              |
| 43 | 1-amino-8-hydroxynaphthalene-3,6-disulfonic acid → 1-amino-2-methoxy-5-methylbenzene → 2-amino-8-hydroxynaphthalene-6-sulfonic acid.                            | alkaline<br>Blue-black.                                                |
| 44 | 1-amino-8-hydroxynaphthalene-3,6-disulfonic acid → 1-amino-2-methoxy-5-methylbenzene → 2-amino-5-hydroxynaphthalene-7-sulfonic acid.                            | alkaline<br>Reddish blue-black.                                        |
| 45 | 1-amino-5-hydroxynaphthalene-7-sulfonic acid → 1-amino-2-methoxy-5-methylbenzene → Cleve's acid.                                                                | alkaline<br>Dark-brown.                                                |
| 46 | 1-amino-5-hydroxynaphthalene-7-sulfonic acid → 1-amino-2-methoxy-5-methylbenzene → 2-amino-8-hydroxynaphthalene-6-sulfonic acid.                                | alkaline<br>Blue-black.                                                |
| 47 | 1-amino-5-hydroxynaphthalene-7-sulfonic acid → 1-amino-2-methoxy-5-methylbenzene → 2-amino-5-hydroxynaphthalene-7-sulfonic acid.                                | alkaline<br>Reddish blue-black.                                        |
| 48 | 1-amino-5-hydroxynaphthalene-7-sulfonic acid → Cleve's acid → Cleve's acid.                                                                                     | Dark-brown.                                                            |
| 49 | 1-amino-5-hydroxynaphthalene-7-sulfonic acid → Cleve's acid → 2-amino-8-hydroxynaphthalene-6-sulfonic acid.                                                     | alkaline<br>Blue-black.                                                |
| 50 | 1-amino-5-hydroxynaphthalene-7-sulfonic acid → Cleve's acid → 2-amino-5-hydroxynaphthalene-7-sulfonic acid.                                                     | Dark-blue.                                                             |
| 51 | 2-amino-8-hydroxynaphthalene-6-sulfonic acid → Cleve's acid → Cleve's acid.                                                                                     | Dark red-brown.                                                        |
| 52 | 2-amino-8-hydroxynaphthalene-6-sulfonic acid → 1-aminonaphthalene → 2-amino-8-hydroxynaphthalene-6-sulfonic acid.                                               | alkaline<br>Black-blue.                                                |
| 53 | 1-amino-7-hydroxynaphthalene → Cleve's acid → Cleve's acid.                                                                                                     | Dark-brown.                                                            |
| 54 | 2-amino-8-hydroxynaphthalene-6-sulfonic acid → 1-(3'-aminophenyl)-5-pyrazolone-3-carboxylic acid<br>alkaline<br>→ 2-amino-8-hydroxynaphthalene-6-sulfonic acid. | Brown.<br>Dark violet-brown.                                           |
| 55 | 2-amino-8-hydroxynaphthalene-6-sulfonic acid → 1-(4'-aminophenyl)-3-methyl-5-pyrazolone<br>2-amino-8-hydroxynaphthalene-6-sulfonic acid.                        | alkaline<br>Brown.                                                     |
| 56 | 2-amino-8-hydroxynaphthalene-6-sulfonic acid → 1-(4'-aminophenyl)-3-methyl-5-pyrazolone → Cleve's acid.                                                         | alkaline<br>Copper-brown.                                              |
| 57 | 2-amino-8-hydroxynaphthalene-6-sulfonic acid → 1-(3'-aminophenyl)-3-methyl-5-pyrazolone<br>2-amino-8-hydroxynaphthalene-6-sulfonic acid.                        | alkaline<br>Blue-black.                                                |
| 58 | 2-amino-5-hydroxynaphthalene-7-sulfonic acid → Cleve's acid → 2-amino-8-hydroxynaphthalene-6-sulfonic acid.                                                     | Dark-brown.                                                            |
| 59 | 2-amino-5-hydroxynaphthalene-7-sulfonic acid → Cleve's acid → Cleve's acid.                                                                                     | Dark-brown.<br>Currant.                                                |
| 60 |                                                                                                                                                                 | Violet-blue.                                                           |
| 61 | 2-amino-5-hydroxynaphthalene-7-sulfonic acid ← 1,4-diaminobenzene ← 2-amino-5-hydroxynaphthalene-7-sulfonic acid.                                               | alkaline<br>Black-violet.                                              |
| 62 | 1-amino-8-hydroxynaphthalene → 2-amino-5-hydroxynaphthalene-7-sulfonic acid → 2-amino-5-hydroxynaphthalene-7-sulfonic acid.                                     | alkaline<br>Blue-black.                                                |
| 63 | 2-amino-8-hydroxynaphthalene-6-sulfonic acid → 1-amino-2-methoxy-5-methylbenzene → 2-amino-8-hydroxynaphthalene-6-sulfonic acid.                                | alkaline<br>Reddish blue-black.                                        |
| 64 | 2-amino-5-hydroxynaphthalene-7-sulfonic acid → 1-amino-2-methoxy-5-methylbenzene → 2-amino-5-hydroxynaphthalene-7-sulfonic acid.                                | alkaline<br>Violet-brown.                                              |
| 65 |                                                                                                                                                                 | Black-violet.<br>Brownish-garnet.                                      |
| 66 | 2-amino-5-hydroxynaphthalene-7-sulfonic acid → 2-(4'-aminobenzoyl-amino)-5-hydroxynaphthalene-7-sulfonic acid.                                                  | Navy-blue.                                                             |
| 67 | 1-(3'-aminophenyl)-3-methyl-5-pyrazolone ← 4,4'-diaminediphenyl-sulfonic acid → 1,8-dihydroxynaphthalene-3,6-disulfonic acid.                                   | Do.<br>Garnet.                                                         |
| 68 | 1-amino-8-hydroxynaphthalene-3,6-disulfonic acid → Cleve's acid → 2-amino-5-hydroxynaphthalene-7-sulfonic acid.                                                 | alkaline<br>Violet-brown.                                              |
| 69 | 1-amino-8-hydroxynaphthalene-3,6-disulfonic acid → Cleve's acid → 2-amino-8-hydroxynaphthalene-6-sulfonic acid.                                                 | alkaline<br>Violet-brown.                                              |
| 70 | 1-amino-8-hydroxynaphthalene-3,6-disulfonic acid → 1-amino-2-methoxy-5-methylbenzene.                                                                           |                                                                        |
| 71 | 1-amino-8-hydroxynaphthalene-5-sulfonic acid → 1-amino-2-methoxy-5-methylbenzene.                                                                               |                                                                        |

|    | Parent dyestuff                                                                                                | Shade on mixed fibers from artificial silk staple fiber and wool |
|----|----------------------------------------------------------------------------------------------------------------|------------------------------------------------------------------|
| 72 | 1-amino-8-hydroxynaphthalene-3,6-disulfonic acid → Cleve's acid                                                | Violet-brown.                                                    |
| 73 | 1-amino-5-hydroxynaphthalene-7-sulfonic acid → 1-amino-2-methoxy-5-methylbenzene                               | Red-brown.                                                       |
| 74 | 1-amino-7-hydroxynaphthalene → Cleve's acid                                                                    | Dark red-brown.                                                  |
| 75 | 2-amino-8-hydroxynaphthalene-6-sulfonic acid → 1-aminonaphthalene                                              | Black-brown.                                                     |
| 76 | 2-amino-5-hydroxynaphthalene-7-sulfonic acid → 1-aminonaphthalene                                              | Brown.                                                           |
| 77 | 2-(4'-aminobenzoyl)amino-8-hydroxynaphthalene-6-sulfonic acid → 1-amino-3,5-dimethylbenzene                    | Garnet.                                                          |
| 78 | 2-amino-8-hydroxynaphthalene-6-sulfonic acid → 1-amino-3,5-dimethylbenzene                                     | Violetish black.                                                 |
| 79 | 2-amino-5-hydroxynaphthalene-7-sulfonic acid → 1-amino-3,5-dimethylbenzene                                     | Do.                                                              |
| 80 | 2-amino-8-hydroxynaphthalene-6-sulfonic acid → meta-amino-acetanilide                                          | Violet-brown.                                                    |
| 81 | 2-amino-8-hydroxynaphthalene-6-sulfonic acid → 1-amino-2-methoxy-5-methylbenzene                               | Reddish black.                                                   |
| 82 | 1-amino-8-hydroxynaphthalene-3,6-disulfonic acid → 1-(3'-aminophenyl)-5-pyrazolone-3-carboxylic acid           | Copper-red.                                                      |
| 83 | 1-amino-2,6-dichloro-4-nitrobenzene → 2-amino-5-hydroxynaphthalene-7-sulfonic acid, reduced                    | Reddish black.                                                   |
| 84 | 1-amino-2,5-dimethoxy-4-nitrobenzene → 2-amino-5-hydroxynaphthalene-7-sulfonic acid, reduced                   | Do.                                                              |
| 85 | 1-amino-2,5-diethoxy-4-nitrobenzene → 2-amino-5-hydroxynaphthalene-7-sulfonic acid, reduced                    | Garnet.                                                          |
| 86 | 1-amino-3-(4'-nitrobenzoyl)-aminobenzene → 2-amino-5-hydroxynaphthalene-7-sulfonic acid, reduced               | Black.                                                           |
| 87 | 1-amino-2-methyl-4-nitrobenzene → 2-amino-5-hydroxynaphthalene-7-sulfonic acid, reduced                        | Black-violet; after treated with a copper compound: black.       |
| 88 | 1-amino-2-methoxy-5-chloro-4-nitrobenzene → 2-amino-5-hydroxynaphthalene-7-sulfonic acid, reduced              | Orange-brown.                                                    |
| 89 | 1-(3'-aminophenyl)-3-methyl-5-pyrazolone ← 4,4'-diamino-diphenyl-sulfonic acid → 1,3-dihydroxybenzene          | Violet-brown.                                                    |
| 90 | 1-amino-8-hydroxynaphthalene → 2-amino-7-hydroxy-naphthalene → 2-amino-5-hydroxynaphthalene-7-sulfonic acid    | Red-brown.                                                       |
| 91 | 1-amino-8-hydroxynaphthalene → 2-(4'-aminobenzoyl-4'-aminobenzoyl-amino)-5-hydroxynaphthalene-7-sulfonic acid  | Do.                                                              |
| 92 | 1-amino-8-hydroxynaphthalene → 2-(3''-aminobenzoyl-4'-aminobenzoyl-amino)-5-hydroxynaphthalene-7-sulfonic acid |                                                                  |

We claim:

1. The process which comprises applying to the fiber an alkali metal salt of a water-soluble azo-dyestuff containing in the molecule an amino-group capable of being diazotized and a hydroxyl group rendering coupling possible, then diazotizing the dyestuff on the fiber and causing it to combine with itself by an alkaline treatment.
2. The process which comprises applying to the fiber an alkali metal salt of a water-soluble azo-dyestuff containing in the molecule an amino-group capable of being diazotized and a hydroxyl group rendering coupling possible, then diazotizing the dyestuff on the fiber and causing it to combine with itself by adding to the diazo-bath an agent having an alkaline action.

3. The process which comprises applying to the fiber an alkali metal salt of a water-soluble azo-dyestuff containing in the molecule an amino-group capable of being diazotized and a hydroxyl group rendering coupling possible, then diazotizing the dyestuff on the fiber and causing it to combine with itself by passing the fiber through a bath having an alkaline action.

4. The process which comprises applying to the fiber an alkali metal salt of a water-soluble azo-dyestuff containing 2-amino-5-hydroxynaphthalene-7-sulfonic acid as azo-component and in the diazo-component an amino-group capable of being diazotized, then diazotizing the dyestuff on the fiber and causing it to combine with itself by an alkaline treatment.

5. The process which comprises applying to mixed fibers from artificial silk staple fiber and wool an alkali metal salt of the water-soluble azo-dyestuff obtainable by coupling diazotized 1-amino-2-hydroxy-4-nitrobenzene in an acid medium with 2-amino-5-hydroxynaphthalene-7-sulfonic acid and reducing the product obtained, corresponding with the following formula:



then diazotizing the dyestuff on the fiber, causing it to combine with itself by an alkaline treatment and treating the dyeing with an agent yielding metal.

6. The process which comprises applying to mixed fibers from artificial silk staple fiber and wool an alkali metal salt of the water-soluble azo-dyestuff obtainable by coupling diazotized 1-amino-2-chloro-4-nitrobenzene in an acid medium with 2-amino-5-hydroxynaphthalene-7-sulfonic acid and reducing the product obtained, corresponding with the following formula:



then diazotizing the dyestuff on the fiber and causing it to combine with itself by an alkaline treatment.

7. The process which comprises applying to mixed fibers from artificial silk staple fiber and wool an alkali metal salt of the water-soluble azo-dyestuff obtainable by coupling diazotized 1-amino-2-chloro-4-nitrobenzene in an acid medium with 2-amino-5-hydroxynaphthalene-7-sulfonic acid and reducing the product obtained, corresponding with the following formula:



then diazotizing the dyestuff on the fiber, causing it to combine with itself by an alkaline treatment and after-chroming the dyeing.

8. The process which comprises applying to mixed fibers from artificial silk staple fiber and wool an alkali metal salt of the water-soluble azo-dyestuff obtainable by coupling diazotized 1-

amino-4-nitrobenzene in an alkaline medium with 2-amino-5-hydroxynaphthalene-7-sulfonic acid, diazotizing the dyestuff obtained, coupling the diazo-compound in an acid medium with 2-phenylamino-5-hydroxynaphthalene-7-sulfonic acid and reducing the product obtained, corresponding with the following formula:



10

amino-4-nitrobenzene in an alkaline medium with 2-amino-5-hydroxynaphthalene-7-sulfonic acid, diazotizing the dyestuff obtained, coupling the diazo-compound in an acid medium with 2-phenylamino-5-hydroxynaphthalene-7-sulfonic acid and reducing the product obtained, corresponding with the following formula:



then diazotizing the dyestuff on the fiber and causing it to combine with itself by an alkaline treatment.

9. The process which comprises applying to mixed fibers from artificial silk staple fiber and wool an alkali metal salt of the water-soluble azo-dyestuff obtainable by coupling diazotized 1-

15

then diazotizing the dyestuff on the fiber, causing it to combine with itself by an alkaline treatment and after-treating the dyeing with a copper-compound.

WERNER KIRST.  
WOLFGANG ALT.  
HANS KRZIKALLA.

20